

R. T. LEE AND T. B. LASHER.

METHOD OF MANUFACTURING ONE-PIECE RUSTLESS KNIVES FOR TABLE USE.  
APPLICATION FILED OCT. 16, 1919.

1,407,794.

Patented Feb. 28, 1922.



Inv. Cutors  
Robert T Lee  
Thomas B Lasher  
or Sigmund Teitel  
atty

# UNITED STATES PATENT OFFICE.

ROBERT T. LEE, OF NORTHAMPTON, MASSACHUSETTS, AND THOMAS B. LASHAR, OF BRIDGEPORT, CONNECTICUT, ASSIGNEES TO INTERNATIONAL SILVER CO., OF BRIDGEPORT, CONNECTICUT, A CORPORATION OF NEW JERSEY.

## METHOD OF MANUFACTURING ONE-PIECE RUSTLESS KNIVES FOR TABLE USE.

1,407,794.

Specification of Letters Patent. Patented Feb. 28, 1922.

Application filed October 16, 1919. Serial No. 331,005.

To all whom it may concern:

Be it known that we, ROBERT T. LEE and THOMAS B. LASHAR, citizens of the United States, residing, respectively, at Northampton, in the county of Hampshire and State of Massachusetts, and at Bridgeport, in the county of Fairfield and State of Connecticut, have invented a new and useful Improvement in Methods of Manufacturing One-Piece Rustless Knives for Table Use; and we do hereby declare the following, when taken in connection with the accompanying drawings and the characters of reference marked thereon, to be a full, clear, and exact description of the same, and which said drawings constitute part of this application, and represent, in—

- Fig. 1 a view of the two blanks before welding.
- Fig. 2 a similar view of the composite blank after the weld.
- Fig. 3 a view of the blank after being drop-forged and before trimming.
- Fig. 4 a view of the completed article.
- Fig. 5 a broken sectional view showing the bolster as a part of the handle.

Our invention relates to a method of manufacturing one-piece rustless knives for table use, such as table knives, carving knives, fruit knives and the like. More specifically our method consists in an improvement upon the method disclosed in U. S. Patent No. 1,020,158 dated March 12, 1912, and granted upon the application of Patrick W. Powers, the object of our present invention being to improve upon the method described in the said Letters Patent, whereby we are enabled to produce knives of superior appearance and wearing qualities at a reduced cost for maintaining the dies used in embossing their handles.

With these ends in view, our invention consists in the method hereinafter described and pointed out in the claims.

In practising our improved method we employ a blade-blank 5 preferably of carbon steel, but our invention is not limited to the use of any particular quality of steel for this blank, the only requirement being that it shall be workable and hardenable. We also employ a handle-blank 6 of a non-ferrous or other rustless metal alloy having a sufficient content of nickel to set up an electrical resistance rising synchronously

with the electrical resistance of the blade-blank. Preferably, for the handle-blank we shall use an alloy of copper and nickel having a sufficiently high content of nickel to meet the electrical requirement above stated, the salient characteristic of our method being the employment of a handle-blank which shall have the characteristic of rising in temperature synchronously with the blade-blank under the action of the welding current. We do not limit ourselves to any specific alloy, but have secured good results with an alloy containing about equal parts of copper and nickel. To this we may add a small amount of zinc for increasing the whiteness and the ductility of the alloy, but the use of zinc may be entirely dispensed with if preferred. Two blanks of the character described and preferably of the same cross section, have their ends abutted under pressure and are then welded at the point of abutment by the passage of the electrical current through them which causes the two metals at the point of abutment to correspondingly rise in temperature until the welding point is reached. The two blanks are thus fused together with the production of a slight flash 7 between them, as shown in Fig. 2. The welded blanks are now subjected to the action of dies whereby the handle 8 and blade 9 are produced. In subjecting the welded blanks to the dies, they are placed therein so that the bolster 10 which is the member between the blade and handle proper, is entirely formed from the handle-blank, since it is the bolster which rests upon the table and takes a heavy portion of the wear upon the knife. When the silver plate covering the bolster is worn away, the wear is not noticeable as the silver-like metal is laid bare rather than the black color exposed when the silver plate is worn away from a steel bolster. The next step in the process is to remove the fin 11 formed by the action of the dies. The handle 8 is now subjected to the action of embossing dies and on account of the relative softness of the metal it may be very deeply and richly embossed to correspond to the embossing on spoons and forks formed from relatively soft metal. On account of the relative softness of the handle-blank the embossing may be deep and intricate without breaking down the edges of the dies.

which are made of hard steel and very costly. We may say in this connection that when the handle-blank is made of a soft steel, such as provided for in the Powers 5 patent referred to, the depth of the embossing is not only very much limited, but the wear on the dies is so great as to be practically prohibitory. We may also state in this connection that when soft steel is employed for the handle as provided for in the Powers patent, the wearing away of the silver-plate from the embossed surface exposes the black color of the steel, rendering the article unsightly. The handle 8 having been embossed, the handle and blade 10 portions of the knife are prepared for the plating operation unless it is desired to leave the blade unplated. On account of the silver-like color of the alloy used for the handle, the knife might be finished and put upon the market without any plating whatever.

By our improved method we are enabled to produce a handsomer and more durable 15 article than can be produced by following the instructions of the Powers patent, as we are enabled to emboss our relatively soft alloy handle more deeply than a soft steel handle, and when the plating wears away in 20 spots, it discloses only a silver-like color hardly distinguishable from the plating. Moreover the embossing of a steel handle rapidly breaks down the costly dies necessary for the purpose and their renewal is 25 a heavy item of expense in carrying on the method of the Powers patent, whereas the soft alloys of our handle blanks not only do not break down the dies but enable very 30 deeply cut dies to be used.

We do not, as already stated, limit ourselves to the employment of any particular 35 quality or composition of steel for the blade-blank, nor any particular alloy for the handle-blank as long as the latter is chosen 40 for a silver-like color and the development of an electrical resistance corresponding to the blade-blank so that the two blanks will rise in temperature together until the melting point is reached.

It will be understood, of course, that as 45 the handle and blade blanks are electrically welded, the resulting article is practically a one-piece article with no perceptible seam or joint to show where one metal blends into 50 the other.

We claim:—

1. A method of producing a one-piece, rustless handle, electrically-welded knife for table use, consisting in abutting under pressure a steel blade-blank and a relatively soft 60 non-ferrous metal handle-blank, the said blanks having substantially the same electrical resistance, whereby they synchronously rise in temperature under the action of a welding current until fusion takes place, 65 then passing a current through the blanks, whereby they are welded together, and then subjecting the welded blanks to the action of dies, whereby they are conformed to knife-shape. 70

2. A method of producing a one-piece, rustless handle, electrically-welded knife for table use, consisting in abutting under pressure a steel blade-blank and a relatively soft 75 non-ferrous metal handle-blank, the said blanks having substantially the same electrical resistance whereby they synchronously rise in temperature under the action of a welding current; then passing a current through the blanks, whereby they are welded together, then subjecting the welded blanks to the action of dies for producing a bolster from the metal of the handle-blank, and finally finishing and electroplating the article. 80

3. A method of producing a one-piece, rustless handle, electrically-welded knife for table use, consisting in abutting under pressure a steel blade-blank and a relatively soft 85 non-ferrous metal handle-blank, the said 90 blanks having substantially the same electrical resistance, whereby they synchronously rise in temperature under the action of a welding current; then passing a current through the blanks, whereby they are welded together; then subjecting the welded blanks to the action of dies for producing a bolster from the metal of the handle-blank; then submitting the knife so produced to the action of embossing dies, and 95 then finishing and electroplating the article. 100

In testimony whereof, we have signed this specification in the presence of two subscribing witnesses.

ROBERT T. LEE.  
THOMAS B. LASHAR.

Witnesses:

CHARLES E. CREGAN,  
MICHAEL W. MOAKLEY.